

May 15, 1934.

P. KNIEPEN

1,958,967

ELECTRON DISCHARGE TUBE AND METHOD OF MAKING SAME

Filed Oct. 21. 1932



INVENTOR  
PETER KNIEPEN  
BY *H. G. Groves*  
ATTORNEY

## UNITED STATES PATENT OFFICE

1,958,967

ELECTRON DISCHARGE TUBE AND METHOD  
OF MAKING SAME

Peter Kniepen, Berlin-Finkenkrug, Germany, assignor to Allgemeine Elektricitat Gesellschaft, Berlin, Germany, a corporation of Germany

Application October 21, 1932, Serial No. 638,896  
In Germany October 22, 1931

6 Claims. (Cl. 250—27.5)

It is known in the prior art that, for the purpose of out-gassing discharge vessels or tubes, metals are disposed in the interior thereof of a kind capable of absorbing gases. More particularly, a method has been disclosed in which, with the said end in view, difficultly meltalble metals such as zirconium are employed in the shape of sheets, ribbons and the like or else in the pulverulent state.

Now, the basic idea of the invention consists in using compounds, more especially hydrides of such metals rather than the pulverulent metals. These are decomposed in outgassing during the pumping process while incidentally resulting in highly reactive metallic powder in a state of extremely fine division. Compounds of the kind here concerned moreover offer this further advantage that they are stable in air.

Their use in practice is very simple. The powder is elutriated in a liquid that is inert in nature and readily evaporable, whereupon such parts as are to be coated, e. g., the anode, are dipped in the said elutriation or paste, or else the latter is applied by spraying or painting. It is particularly the hydride form of compound that has proved especially suitable seeing that the hydrogen which is evolved during outgassing process, as is well known in the art, promotes and expedites to a large degree the completion of the outgassing operation, cleaning of electrodes, etc. Particularly useful was found to be, for instance, a paste prepared with zirconium hydride and readily volatilizable hydrocarbons such as xylene with an addition or admixture of a substance with a high boiling point such as paraffin.

It may also be advantageous to use as the support for the porous layer a sort of metal such as nickel which is capable of alloying itself with the ensuing porous metal such as zirconium, because this promotes the adhesiveness upon the substratum.

It may furthermore be of advantage to use mixtures of compounds of such metals, such as tantalum or zirconium, as will in practical use fail to form mixed crystals, in order to preclude in spite of high loads the sintering of the porous layer with an incidental loss of its porous properties and gas absorptiveness.

Occasionally it may be advantageous, with a view to promote the adhesiveness of the active metal upon the substratum, to roughen the latter or to provide it with a porous coat consisting of the same metal or some other metal, such as nickel. For the identical reason it is advantageous to priorly anneal (thoroughly heat) the metal parts to be treated in an atmosphere of pure hydrogen.

It has also been discovered that gas-absorbent metallic powders such as zirconium, titanium, vanadium and niobium, possess a higher heat

radiation than bare polished metals and also that their radiation powers are not appreciably altered in the course of relatively long periods of operating time. According to the invention powders of the said sort, say, zirconium powder, are prepared in paste form as above described and are applied to the anode by spraying or painting. The result is that the load-carrying capacity of the tube can be greatly increased, with the consequence that far smaller dimensions may be chosen for the anode and thus for the whole tube conjointly with a chance of using metals that had heretofore been unserviceable for the present purpose, under like load conditions, such as nickel. It has been discovered that in the case of a nickel anode coated as above it is able to carry a specific load of from 6 to 8 watts per sq. cm. and over, as contrasted with 2-3 watts per sq. cm. in the case of uncoated nickel anodes, and 4-5 watts per sq. cm. for tantalum anodes. The load capacity is further increasable if instead of nickel, molybdenum, tungsten or tantalum is used as the supporting or substratum material.

What is claimed is:

1. In the art of gettering an evacuated envelope, the method which consists in introducing the solid hydride of a gettering material into the envelope before evacuation, heating the material, and evacuating the envelope to remove the evolved hydrogen whereby said material is changed into a porous mass capable of absorbing large quantities of deleterious gases.

2. In the art of gettering an evacuated envelope containing a support member, the method which consists in coating the member with the hydride of a gettering material, heating said member to remove the hydrogen from the material and to obtain a porous metal coating capable of absorbing large quantities of deleterious gases.

3. In the art of gettering an evacuated envelope containing electrodes, the method which consists in depositing zirconium hydride on one of the electrodes, heating the coated electrode and removing the evolved hydrogen to obtain a residue layer in finely divided form capable of absorbing large quantities of deleterious gases.

4. The method of improving the heat radiating qualities of anode electrodes in electron discharge tubes, which comprises coating the anode with zirconium hydride.

5. An electron discharge tube having a metallic anode, and a hydride compound coated on said anode and capable of alloying therewith.

6. An electron discharge tube having an anode of nickel, and a zirconium hydride compound capable of alloying with said nickel anode coated thereon.

PETER KNIEPEN.

120